

[72] Inventors **Irving W. Wolf**  
 Palo Alto, Calif.;  
**David Treves, Rehovoth, Israel; Nathan**  
**Ballard, Santa Clara, Calif.**  
 739,602  
 [21] Appl. No.  
 [22] Filed May 13, 1968  
 [45] Patented Oct. 5, 1971  
 [73] Assignee **Ampex Corporation**  
 Redwood City, Calif.

[56] **References Cited**  
 UNITED STATES PATENTS  
 3,364,496 1/1968 Greiner et al. .... 346/74  
 3,463,708 8/1969 Grant ..... 204/43  
 Primary Examiner—Bernard Konick  
 Assistant Examiner—Gary M. Hoffman  
 Attorney—Robert G. Clay

[54] **THERMOMAGNETIC RECORDING PROCESS**  
 4 Claims, 1 Drawing Fig.  
 [52] U.S. Cl. .... 346/74,  
 117/238, 179/100.2, 204/43  
 [51] Int. Cl. .... G01d 15/12,  
 C23b 5/32  
 [50] **Field of Search** .... 346/74 M,  
 74 MT, 74 MP; 179/100.2 CF, 100.2 CR; 117/235,  
 238; 204/43; 250/65.1; 340/174 TF, 174

**ABSTRACT:** A recording process is provided for a thermomagnetic recording system wherein recording is by a combination of heating and magnetization of a medium which consists largely of cobalt in hexagonal form. The medium is plated from a cobalt electrolyte containing a small amount of phosphorous at a pH of from 5.5 to 6.6. A small amount of nickel may also be present. The resulting recording medium has strongly temperature dependent coercivity characteristics at temperatures well below the Curie point and the ratio of coercivity at 15°C. to that at 150°C. is at least two.



PATENTED OCT 5 1971

3,611,416



INVENTORS  
IRVING W. WOLF,  
DAVID TREVES &  
NATHAN BALLARD  
BY  
*Robert S. Clay*  
ATTORNEY

## THERMOMAGNETIC RECORDING PROCESS

### BACKGROUND OF THE INVENTION

#### 1. Field of the Invention

Thermomagnetic recording process.

#### 2. Description of the Prior Art

The materials heretofore available for thermomagnetic recording were relatively inefficient and required high-recording temperatures. The present invention differs from the prior art in the use of materials having a high ratio of coercivity at normal temperatures to relatively low elevated temperatures, i.e., well below the Curie point.

### SUMMARY OF THE INVENTION

Various recording techniques utilizing a combination of heating and magnetism have been known in the past. One typical system utilizes an electron beam to locally heat a magnetized film to the Curie temperature, causing the coercivity of the heated spot of film to decrease, permitting the reversal of magnetism therein by a relatively weak field. Ordinarily temperatures as high as 1,000° C. are required. Typical temperature thermowrite devices are described in U.S. Pat. Nos. 3,176,278 and 2,915,594. Another thermal system utilizes garnet materials to accomplish thermal writing at a temperature near the compensation point at which the average magnetic moment of the materials goes to zero. Other proposed systems utilize the combination of thermally induced stress and magnetostriction effects to provide recording while others employ radiation with ultraviolet light to change the magnetic moment of gadolinium iron garnets.

In pending application, Ser. No. 622,795 now U.S. Pat. No. 3,521,294 an improved magnetothermal recording method is disclosed wherein writing is achieved by locally heating an anomalous medium while simultaneously magnetizing it, said heating being at a temperature substantially below that of the Curie temperature region.

The present invention provides improved materials for such a low temperature thermal recording system which operates efficiently at temperatures as low as 150° to 200° C. while prior art materials utilizing the Curie effect must operate at temperatures on the order of 1,000° C. Because of the low temperature involved and the short heating time, the use of plastic substrates is entirely practical.

### BRIEF DESCRIPTION OF THE DRAWING

The sole FIGURE of the drawing is a graph showing the decrease in coercivity of a material prepared in accordance with example 1 of the present invention. It shows that the material has a coercivity of about 450 Oe at room temperature and that the coercivity has fallen to about one-fourth of its former value at 150° C. and to about one-sixth at 200° C.

### DESCRIPTION OF THE PREFERRED EMBODIMENTS

Copending patent application Ser. No. 622,795 describes in detail the utilization of materials having anomalous thermomagnetic properties. In general, the method consists of providing a heat-generating field such as an electric heater or an electron beam source which is focused on a small portion of the recording medium. Simultaneously, a weak magnetic field is applied to the same portion of the recording medium. Either the heat beam or the magnetic field, or both, can be modulated to record the desired information on the recording medium.

In accordance with the present invention, it has been found that a highly effective low-temperature thermal writing process can be provided by electroplating a film containing predominately cobalt with a small amount of phosphorus and optionally a small amount of nickel. If such plating were conducted in accordance with normal practice, i.e., using a relatively low pH, ordinary cubic cobalt would be deposited and the anomalous behavior desired, i.e., a highly sensitive temperature dependent coercivity, would not be achieved. In ac-

cordance with the present invention, it has been found that if the plating is conducted at a high pH, i.e., from 5.5 to 6.6 or preferably from 6 to 6.6, cobalt is not deposited in the cubic form, but is deposited in a hexagonal form, yielding a recording medium having the desired temperature-sensitive coercivity. If the pH of the plating solution is below 5.5 the cubic form is deposited, defeating the purpose of the present invention while 6.6 is given as an upper limit only because at a higher pH there will normally be precipitation of the salts from the plating solution; this is ordinarily undesirable since any solid, suspended matter in the plating solution might interfere with the deposit of a smooth, even coating.

By following the technique of the present invention, it is easy to achieve ratios of coercivity of 2:1 and even as high as 4:1 as is shown in example 1 in the drawing. By ratio, is meant the ratio of the coercivity of the material at about room temperature, i.e., 15° C. and at a temperature of 150° C. In addition, the coercivities of the materials are well over 100 at room temperature, yielding a satisfactory output and rendering them more or less immune to print through self-demagnetizing effects at workable densities or changes in magnetization due to small, stray magnetic fields. The materials utilized in the process of the present invention also have an excellent squareness or remanence ratio ( $Br/Bs$ ) as is shown by the data wherein all of the materials of the present invention have a squareness of better than 0.8.

Various salts can be used in the plating bath and, as the examples shows, the effects are not dependent upon the anions in the bath. Thus, there can be mixtures of sulfate and chloride, all sulfate, all chloride, or sulfamate, for example without substantially affecting the process of the present invention.

The plating conditions can vary over wide limits. Although it is normally preferred to operate at a current density of about 100 ma. per square inch, current densities as low as 5 ma. may be employed although at these low-current densities plating takes place so slowly that it is not economically desirable. The current density can go as high as 500 ma. per square inch but at higher densities the coating tends to become grainy and therefore less useful.

The change in coercivity upon heating is almost completely reversible as is shown in the working examples. Thus, when the plating of the present invention was heated to 150° C. and held at this temperature for 10 minutes, the coercivity returned to almost its former value when the material was cooled to 15° C.

The concentration of the materials on the plating bath is ordinarily not critical so long as the concentration is not made so great or the pH raised to the point where materials precipitate from the bath.

The ratio of phosphorus (as hypophosphite) to cobalt in the bath can vary from about 0.08/100 to 2.3/100 by weight and the concentration in nickel can vary from 0/100 to 10/100. The metallic ions do not plate out in direct proportion to their concentration in the bath, the proportions being approximately 1.5 to 1 in the case of phosphorus and approximately 4 to 1 in the case of nickel. Therefore with respect to the plating itself as distinguished from the bath, the plate itself can contain from approximately 0.05 to 1.5 percent phosphorus and from 0 to 2.5 percent nickel by weight, the balance being cobalt.

The nature of the substrate is not critical so long as it is non-magnetic, conductive and has a smooth surface. Thus metals such as brass or aluminum can be used as well as nonconductors having a conductive surface which can be deposited by vacuum evaporation or electroless methods. Plastics such as polyesters, polyolefins and cellulose acetate are all suitable.

The following nonlimiting examples illustrate preferred embodiments of the invention:

### EXAMPLE I

A film was electrodeposited on a sputtered gold-on-polyester substrate from a bath of the following composition:

|                                                  |           |
|--------------------------------------------------|-----------|
| Cobalt sulfate (hydrate)                         | 200 g./l. |
| Sodium chloride                                  | 10 g./l.  |
| Sodium hypophosphite                             | 0.3 g./l. |
| Boric acid                                       | 15 g./l.  |
| Sodium lauryl sulfate (wetting agent)            | 5 g./l.   |
| pH=6.0, adjusted with sodium hydroxide solution. |           |

Plating was carried out at room temperature at a cathode current density of 50 ma./in.<sup>2</sup>. This film's thermomagnetic properties are plotted in the drawing showing temperature vs coercive force for a 200 A. thick magnetic film. The plating was composed of 99.9 percent cobalt and approximately 0.1 percent phosphorus by weight.

## EXAMPLE II

| Bath composition                                   |           |
|----------------------------------------------------|-----------|
| CoSO <sub>4</sub> ·7H <sub>2</sub> O               | 200 g./l. |
| H <sub>3</sub> BO <sub>3</sub>                     | 15 g./l.  |
| NaCl                                               | 25 g./l.  |
| NaC <sub>12</sub> H <sub>25</sub> SO <sub>4</sub>  | 5 g./l.   |
| NaH <sub>2</sub> PO <sub>2</sub> ·H <sub>2</sub> O | 0.3 g./l. |
| pH=6                                               |           |

|                       |          |
|-----------------------|----------|
| Boric acid            | 15 g./l. |
| Sodium lauryl sulfate | 5 g./l.  |
| NaCl                  | 25 g./l. |

## EXAMPLE VI

|                 |                                                    |             |
|-----------------|----------------------------------------------------|-------------|
| Sulfamate bath: | Co sulfamate                                       | 157.5 g./l. |
|                 | NaH <sub>2</sub> PO <sub>2</sub> ·H <sub>2</sub> O | 0.3 g./l.   |
|                 | Boric acid                                         | 15 g./l.    |
|                 | Sodium lauryl sulfate                              | 5 g./l.     |

## EXAMPLE VII

|                   |                                                    |           |
|-------------------|----------------------------------------------------|-----------|
| All sulfate bath: | CoSO <sub>4</sub> ·7H <sub>2</sub> O               | 200 g./l. |
|                   | NaH <sub>2</sub> PO <sub>2</sub> ·H <sub>2</sub> O | 0.3 g./l. |
|                   | Boric acid                                         | 15 g./l.  |
|                   | Sodium lauryl sulfate                              | 5 g./l.   |

The characteristic of the platings are given in the following table:

| Example  | Anions                | H <sub>c</sub><br>15° C.<br>(BH) | H <sub>c</sub><br>150° C.<br>(BH) | H <sub>c</sub><br>15° C.<br>(AH) | Ratio | Thickness,<br>A. | Remain-<br>ance,<br>Br/B <sub>0</sub> |
|----------|-----------------------|----------------------------------|-----------------------------------|----------------------------------|-------|------------------|---------------------------------------|
| I.....   | Sulfate chloride..... | 226                              | 88                                | 190                              | 2.57  | 100              | .864                                  |
|          | do.....               | 270                              | 85                                | 272                              | 3.18  | 200              | .816                                  |
| V.....   | All chloride.....     | 245                              | 81                                | 224                              | 3.02  | 100              | .850                                  |
|          | do.....               | 339                              | 94                                | 344                              | 3.61  | 200              | .833                                  |
| VI.....  | Sulfamate.....        | 196                              | 76                                | 170                              | 2.56  | 100              | .881                                  |
|          | do.....               | 228                              | 73                                | 233                              | 3.12  | 200              | .824                                  |
| VII..... | All sulfate.....      | 210                              | 72                                | 209                              | 2.92  | 100              | .835                                  |
|          | do.....               | 280                              | 81                                | 290                              | 3.46  | 200              | .825                                  |

BH=before heating.

AH=after heating for 10 minutes at 150° C.

Ratio=coercivity at 15° C. divided by coercivity at 150° C.

Plating was conducted at 5 ma./in.<sup>2</sup> to a thickness of 200 A. on a nonmagnetic conductive substrate.

The plating had the following characteristics:

H<sub>c</sub> at 12° 445 Oe  
H<sub>c</sub> at 150° 115 Oe  
H<sub>c</sub> at 200° 90 Oe

## EXAMPLE III

The process of example I was repeated except that the amount of phosphorus was changed to 3.0 g./l. NaH<sub>2</sub>PO<sub>2</sub>·H<sub>2</sub>O and the current density was 500 ma./in.<sup>2</sup>.

The plating had the following characteristics:

H<sub>c</sub> at 12° 294  
H<sub>c</sub> at 150° 97  
H<sub>c</sub> at 200° 61

## EXAMPLE IV

The process of example I was repeated except that the amount of phosphorus was changed to 1.0 g./l. NaH<sub>2</sub>PO<sub>2</sub>·H<sub>2</sub>O and there was added 9.5 g./l. NiSO<sub>4</sub>·6 H<sub>2</sub>O. Also the current density was 100 ma./in.<sup>2</sup>.

The plating had the following characteristics:

H<sub>c</sub> at 12° 273  
H<sub>c</sub> at 150° 95  
H<sub>c</sub> at 200° 63

In the above examples, the anions present in the plating bath were a combination of sulfate and chloride. However the process is not anion-dependent as the following examples V through VII show. In each instance the bath was maintained at 15° C., plating was conducted at a current density of 200 ma./in.<sup>2</sup>, and the pH was adjusted to 6.55. Plating thickness was 100 A. and 200 A.

## EXAMPLE V

Chloride bath: CoCl<sub>2</sub>·6H<sub>2</sub>O  
NaH<sub>2</sub>PO<sub>2</sub>·H<sub>2</sub>O

45 15° C. 165 Oe 88 Oe  
Cobalt alone 334 Oe 88 Oe

50 Thus, although the phosphorus had no substantial effect on coercivity at the elevated temperature, it had a very substantial effect on coercivity at room temperature.

We claim:

1. In a process for thermomagnetic recording of information on a recording medium which is responsive to heat, wherein the medium is scanned by a heat-producing beam while applying a selected magnetic field thereto while maintaining the heat produced by the beam at an elevated temperature substantially below the Curie temperature to produce a decrease in coercivity of the medium to render same responsive to the applied magnetic field and the beam and the applied field define the means for selectively introducing the information to be recorded, the improvement comprising employing as the medium a plating on a nonmagnetic substrate wherein the plating is predominately cobalt with from 0.05 to 1.5 percent by weight phosphorus, said plating being in the hexagonal form.

2. The process of claim 1 wherein the coating contains up to 2.5 percent nickel.

3. The process of claim 1 wherein the plating is deposited from a bath maintained at a pH of from 5.5 to 6.6.

4. The process of claim 1 wherein the plating has a coercivity of at least 100 Oe and has a ratio of coercivity at 15° C. divided by the coercivity at 150° C. of at least 2.